

Feb. 11, 1936.

B. C. BREN

2,030,568

LAMINATED RECORD

Filed Dec. 6, 1933

Fig. 1



Fig. 2



Fig. 3



INVENTOR.  
*Borzech C. Bren*  
BY

*J. M. Castle Jr.*  
ATTORNEY.

## UNITED STATES PATENT OFFICE

2,030,568

## LAMINATED RECORD

Bozotech C. Bren, Cedar Grove, N. J., assignor  
to Dupont Viscoloid Company, Wilmington,  
Del., a corporation of Delaware

Application December 6, 1933, Serial No. 701,110

6 Claims. (Cl. 154—43)

This invention relates to laminated records and the method of making same and, more particularly, to a sound record composed of a relatively thick core upon which is superposed on one or both sides a thin playing surface into which surface a sound groove is impressed.

Heretofore records on which vibratory motion is recorded by means of grooves, and particularly sound records, have been made both as a single, homogeneous composition throughout and as a laminated structure having a relatively thick core of one material and a thin playing surface on one or both sides in the case of a disk record, or merely on the outside in the cylindrical type of record.

Where records of the laminated type have been made, this has been done for the purpose of improving the mechanical strength of the record and also for the purpose of combining the superior acoustical or wearing properties of one material with the greater strength or cheapness of another material. Although many improvements have been made in records of this type, there has not, as yet, been provided an entirely satisfactory laminated record having good acoustical properties and yet relatively economical to manufacture.

An object of the present invention is to provide a laminated record which is inexpensive and yet possesses properties as good as, or better than, any record heretofore known. A further object is to provide a sound record having superior acoustical properties at a reasonable cost. A still further object is to provide an economical and simple process of manufacturing laminated records having advantageous properties.

The above objects are accomplished according to the present invention by making a record having a relatively thick core of a filled cellulose derivative composition and superposed thereon a thin playing surface of an unfilled cellulose derivative composition. Where a disk record is desired having two playing surfaces, a thin playing surface of an unfilled cellulose derivative composition will be superposed on both sides of the core.

Preferred embodiments of the invention are illustrated in the accompanying drawing, wherein Fig. 1 is an enlarged and diagrammatical cross section of a fragment of a disk record having one playing surface, Fig. 2 is a similar view of a fragment of a disk record having two playing surfaces, and Fig. 3 is a similar view parallel to the longitudinal axis of a cylindrical record which, of course, has only one playing surface.

Referring to the drawing, reference numeral 1 designates the relatively thick core of the record which, according to the present invention, is composed of a filled cellulose derivative composition; 2 represents the relatively thin playing surface superposed on the core and composed of an unfilled cellulose derivative composition, and 3 represents the sound grooves customarily made on records of this type.

Through extensive research on sound records made of various compositions, it has been found that cellulose derivatives and in particular cellulose acetate, have unique excellence as material for sound records in that the recordings impressed therein, when played, have been found to have a distinctly superior degree of faithfulness to the original sound and an exceptional freedom from extraneous noise. The superior faithfulness of reproduction possible with these substances is probably attributable to their excellent flowing and molding properties, which enable them to receive a very accurate and exact duplication of the sound recording from the matrix. The freedom from extraneous noise in reproduction, i. e., the absence of so-called scratch, or surface, or background noise, is due probably to the complete homogeneity of such material and its freedom from gritty or brittle constituents. Although the present invention is applicable to cellulose derivative compositions in general, the cellulose acetate compositions, due to their superiority, are preferred, and accordingly the present invention is specifically described with respect to this particular ester. However, in place of cellulose acetate, the other well known cellulose derivatives, such as cellulose nitrate, propionate, or the various ethers, such as ethyl cellulose, benzyl cellulose, and similar ethers, may be employed.

Although it has been discovered that cellulose acetate is outstandingly suitable for the manufacture of high grade sound records, this compound is subject to the objection of hygroscopicity, with the result that a thin sheet record of cellulose acetate composition is subject to the disadvantage of warping with changes in atmospheric conditions. It is desirable, therefore, that records of cellulose acetate composition be made of relatively large thickness and this results in a rather high material cost per record where a homogeneous cellulose acetate record with no filler, or very little filler, is used.

According to the present invention, it has been found that the unparalleled acoustical advan-

ages of unfilled cellulose acetate composition may be retained absolutely unimpaired, but nevertheless the cost of the record appreciably reduced, by using instead of a solid, homogeneous record of 5 unfilled cellulose acetate composition, a laminated record comprising a core molded from a cellulose acetate composition of high filler content and then superposing on said core a relatively thin playing surface composed of an unfilled cellulose acetate composition. The method of manufacturing these records is subject to wide variation, but it is preferred to make up the filled cellulose acetate composition as a powder and mold it according to well known methods by the 10 application of heat and pressure in a suitable die to form the core, and then to superpose on one or both sides of said core a thin layer or sheet of the unfilled cellulose composition and weld the two laminations together by the application of heat and pressure. This is accomplished 15 preferably in the customary record die proper so that the application of the thin playing surface to the core and the imprinting of a sound recording upon the playing surface may be accomplished 20 simultaneously. However, it is obvious that the playing surface and core may be welded together in a die having no sound recording thereon, thereby producing a blank record upon which the sound recording may be impressed at a later time 25 30 in a separate operation.

The molding and processing operations herein referred to have been long known to the art and those skilled in this art would readily understand that, depending upon the specific formula of the 35 compositions used, conditions of pressure and temperature will be varied in accordance with known practice. However, it should be noted that these cellulose acetate compositions used both for the core and the thin playing surface are thermoplastic and may be welded together merely by the application of heat and pressure without the use of auxiliary adhesives and, in the preferred embodiment of the invention, the record is made 40 45 in this manner because the finished article is appreciably better in acoustical properties and freedom from warpage.

The core material, according to the present invention, is composed essentially of cellulose acetate, plasticizer, and a relatively high proportion of filler, the latter greatly reducing the material cost of the record and, if anything, improving the quality of the record.

50 55 The following examples are given to illustrate specific formulas of material adapted for use in the core, parts being given by weight:

*Example 1*

|                      | Parts |
|----------------------|-------|
| 60 Cellulose acetate | 100   |
| Triphenyl phosphate  | 17    |
| Dimethyl phthalate   | 25    |
| Wood flour           | 100   |
| 65 Pigment           | 17    |

*Example 2*

|                           | Parts |
|---------------------------|-------|
| 70 Cellulose acetate      | 100   |
| Triphenyl phosphate       | 25    |
| Dimethoxy ethyl phthalate | 42    |
| Wood pulp                 | 67    |
| China clay                | 83    |
| 75 Pigment                | 17    |

*Example 3*

|                             | Parts |
|-----------------------------|-------|
| Cellulose acetate           | 100   |
| Triphenyl phosphate         | 19    |
| p-Toluene sulfonamide       | 15    |
| Ethyl p-toluene sulfonamide | 19    |
| Cottonseed hull fiber       | 123   |
| Pigment                     | 6     |

*Example 4*

|                           | Parts |
|---------------------------|-------|
| Cellulose acetate         | 100   |
| Triphenyl phosphate       | 10    |
| Dimethoxy ethyl phthalate | 40    |
| Wood flour                | 75    |
| China clay                | 75    |
| Pigment                   | 12    |

*Example 5*

|                           | Parts |
|---------------------------|-------|
| Cellulose acetate         | 100   |
| Triphenyl phosphate       | 12    |
| Dimethoxy ethyl phthalate | 50    |
| Wood flour                | 100   |
| China clay                | 100   |
| Pigment                   | 25    |

*Example 6*

|                           | Parts |
|---------------------------|-------|
| Cellulose acetate         | 100   |
| Triphenyl phosphate       | 12    |
| Dimethoxy ethyl phthalate | 32    |
| Wood flour                | 286   |
| Pigment                   | 9     |

It is preferred that in these compositions for the core, the following range of proportions be observed (parts by weight):—

|                   | Parts      |
|-------------------|------------|
| Cellulose acetate | 100        |
| Plasticizer       | 44 to 62   |
| Filler            | 123 to 286 |

It will be understood that the above examples are merely illustrative and that in place of the common plasticizers disclosed above, other plasticizers well known in the cellulose acetate art may be employed, as well as various mixtures of such plasticizers. Likewise, other fillers may be employed, although it has been found that wood flour is a satisfactory and preferred filler. With respect to the proportions in the core composition, these may be varied considerably as is well known in the art. In order to effect any appreciable economy in the cost of material used in the record, the percentage of filler should be high, and preferably this should range from a ratio of 100 parts by weight of cellulose acetate to 75 to 300 parts by weight of filler, the preferred formula for records of a certain type being readily determined according to the ordinary practice in the cellulose derivative plastic art. The addition of pigment is usual in such compositions but is not necessary.

The following examples illustrate typical formulas for the cellulose acetate material to be used in the thin playing surface, parts being given by weight:—

*Example 7*

|                     | Parts |
|---------------------|-------|
| Cellulose acetate   | 80    |
| Triphenyl phosphate | 8     |
| Dimethyl phthalate  | 12    |

## Example 8

|                             | Parts |
|-----------------------------|-------|
| Cellulose acetate           | 75    |
| Triphenyl phosphate         | 10    |
| 5 Dimethoxy ethyl phthalate | 15    |

## Example 9

|                                | Parts |
|--------------------------------|-------|
| Cellulose acetate              | 70    |
| p-Toluene sulfonamide          | 20    |
| 10 Ethyl p-toluene sulfonamide | 10    |

## Example 10

|                        | Parts |
|------------------------|-------|
| Cellulose acetate      | 85    |
| 15 Triphenyl phosphate | 7     |
| Triacetin              | 8     |

It is preferred that in these compositions for the playing surface the following range of proportions be observed (parts by weight):—

|                   | Parts      |
|-------------------|------------|
| Cellulose acetate | 100        |
| Plasticizer       | 43 to 17.5 |

It will be noted that in the above examples no filler is used, and therefore, that the playing surface of the records according to the present invention is essentially composed of a cellulose derivative, preferably the acetate, and a plasticizer. A small amount of coloring matter may be employed if desired. As those skilled in this art will understand, not only the plasticizers disclosed in the above examples may be used, but other plasticizers known in this art may be substituted in part or wholly, and likewise mixtures of such plasticizers may be used. The proportion of plasticizer to cellulose acetate will be varied in order that the exact degree of hardness and flexibility desired for making records of particular types may be obtained.

According to this invention, the unfilled cellulose acetate compositions illustrated above are worked up into sheet form according to usual practices and used as such in making the laminated record, whereas it is preferred to make the core by using the filled molding material as a powder, although sheets or fragments may likewise be used to fill the mold wherein the core is to be made by the application of heat and pressure.

In the drawing forming part of the present application, no attempt has been made to accurately show the overall thickness or the exact relative thickness of the laminations of the record.

Generally, the total thickness of a disk record whose diameter is 12" will ordinarily be at least  $\frac{1}{8}$  of an inch, whereas the thickness of the playing surface is preferably not less than 1/100 of an inch. In the preferred form of the invention the thickness of the playing surface is substantially greater than the depth of the sound groove, as the acoustical properties of the record are considerably improved if the thickness of the playing surface is great enough so that when the sound groove is impressed upon the playing surface the groove will not be transmitted by the playing surface through to the core to any appreciable extent.

The specific examples of compositions have been given with respect to cellulose acetate, but it is to be understood that the invention in its broader phases also includes the use of other cellulose derivative compositions and the formulation of specific compositions of the other cellu-

lose derivatives involves no more than the skill of the ordinary worker in this art, as long as the essential features of the invention are observed, namely, that the core material be highly filled, whereas the material to be used as a playing surface be an unfilled composition.

The present invention is directed primarily to the production of sound records of the disk type, but it is to be understood that it is also applicable to any other technique in which vibratory motion is recorded by means of grooves. It is by no means necessary that the record be in disk form, as the invention is equally applicable to the commonly used cylindrical records.

An advantage of the present invention lies in the fact that the herein described laminated records secure the superior acoustical advantages of a relatively thick record of an unfilled cellulose acetate composition without the excessive cost of such a record, this being due to the fact that the use of a highly filled molding composition with a base of cellulose acetate as the core of the record has the unexpected result of leaving unimpaired the acoustical advantages of the unfilled cellulose acetate playing surfaces. This advantage is likewise true, although to a more limited extent, in records made from other cellulose derivative compositions. The fact that the acoustical properties of the unfilled cellulose acetate playing surface remain unimpaired is most unexpected, since a laminated record made with a cellulose acetate playing surface but a core other than a cellulose acetate filled composition core badly impairs the acoustical advantages of the playing surface. Likewise, if the playing surface is not appreciably thicker than the depth of the sound groove the acoustical properties of the record are also impaired. Another advantage of the herein described records lies in the fact that adhesion of the laminations is obtained by the application of heat and pressure alone, and this omission of auxiliary adhesive not only provides a more economical process in laminating, a step in the composite operation, but also has the advantage of eliminating a frequent cause of warpage.

In both the molding of the core and the welding of the sheet forming the playing surface to the core, the heat and pressure employed will be varied considerably as the formulation of the compositions is changed. However, it has been found that a pressure of about 1500 to 3000 pounds per square inch and a temperature of 130 to 175° C. is usually satisfactory. It will be understood that the present invention is not to be limited to such temperatures and pressures and, in its broader phases, even includes the use of an auxiliary adhesive whereby the laminations may be united without employing heat at all.

As many apparently widely different embodiments of this invention may be made without departing from the spirit and scope thereof, it is to be understood that the invention is not limited to the specific embodiments thereof except as defined in the appended claims.

I claim:

1. A laminated sound record comprising a relatively thick core of a homogeneous cellulose acetate composition containing finely divided filler and a thin playing surface of an unfilled cellulose acetate composition.

2. A laminated sound record comprising a relatively thick core of a homogeneous cellulose acetate composition containing finely divided filler and a thin playing surface of an unfilled cellulose

acetate composition, said core and playing surface being united without an intermediate adhesive layer.

3. A laminated sound record comprising a relatively thick core of a homogeneous cellulose acetate composition containing finely divided filler and a thin playing surface of an unfilled cellulose acetate composition, said core and playing surface being united without an intermediate adhesive layer and the thickness of said playing surface being appreciably greater than the depth of the sound groove impressed thereon.

4. A laminated sound record comprising a relatively thick core composed essentially of cellulose acetate, plasticizer, and uniformly distributed finely divided filler, and a thin playing surface composed essentially of cellulose acetate and plasticizer.

5. A laminated sound record comprising a relatively thick core composed essentially of cellulose acetate, plasticizer, and uniformly distributed finely divided filler, and a thin playing surface composed essentially of cellulose acetate and plasticizer, said core and playing surface being united without an intermediate adhesive layer.

6. A laminated sound record comprising a relatively thick core composed essentially of cellulose acetate, plasticizer, and uniformly distributed finely divided filler, and a thin playing surface composed essentially of cellulose acetate and plasticizer, said core and playing surface being united without an intermediate adhesive layer and the thickness of said playing surface being appreciably greater than the depth of the sound groove impressed thereon.

BOZETECH C. BREN.